

Aug. 19, 1952

W. G. REYNOLDS

2,607,109

METHOD FOR PRODUCING ALUMINUM-ARMORED CABLES

Filed July 13, 1949

2 SHEETS—SHEET 1



INVENTOR.

William G. Reynolds  
BY  
H. Lee Nelson  
Attorney

Aug. 19, 1952

W. G. REYNOLDS

2,607,109

## METHOD FOR PRODUCING ALUMINUM-ARMORED CABLES

Filed July 13, 1949

2 SHEETS—SHEET 2



## UNITED STATES PATENT OFFICE

2,607,109

## METHOD FOR PRODUCING ALUMINUM-ARMORED CABLES

William G. Reynolds, Louisville, Ky., assignor to Reynolds Metals Company, a corporation of Delaware

Application July 13, 1949, Serial No. 104,555

3 Claims. (Cl. 29—155.42)

1

The object of this invention is to provide an effective method for producing aluminum armored steel cable, that is to say, a composite cable, in which the application of the aluminum to the generally ferrous core is effected by pressure welding at high speed, and in such manner that many aluminum armored cables may be produced simultaneously, with the armoring aluminum initially in the form of opposed sheets which blanket the cables. These sheets will in practice be webs fed from coils through cleansing, pre-forming, heating, pressure, slitting, and drawing zones. The invention is, of course, applicable to the encasing or armoring of strands having various gauges and composed of various metals.

The invention will be described with reference to the accompanying drawing in which:

Fig. 1 is a schematic view in elevation, indicating the stations and elements through which the aluminum sheet webs and the wire or cables are passed.

Fig. 1a is a fragmentary plan view, taken at the feed-end of the machine, the aluminum uppermost sheet being broken away.

Fig. 2 is a view in elevation showing a set of the wire guiding rolls.

Fig. 3 is a view in elevation showing a set of the pre-forming rolls for the top aluminum sheet or web.

Fig. 4 is a fragmentary view in elevation showing the welding rolls, with wire strands between them, portions of the backing rolls, and upper and lower aluminum sheets, the latter being shown in section.

Fig. 5 is a fragmentary view in elevation showing one form of the slitter wheels and their action.

Fig. 6 is a view in side elevation of the elements shown in the preceding figure.

Fig. 7 is a view in transverse section showing a group of wires encased by the upper and lower aluminum sheets, prior to separation by slitting.

Fig. 8 is a view similar to Fig. 7 showing the separated encased wires preliminary to their passage through drawing or forming dies to remove the lips.

Fig. 9 is a cross section taken through an encased completed cable.

Fig. 10 is a fragmentary view in section showing one formation of the two aluminum sheets before the welding operation and at an area for encasing two wires.

Fig. 11 is a view similar to Fig. 10 showing the said sheet areas in their subsequent welded form.

2

To initially show the nature of the process and the elements employed, reference may be made to Fig. 1, which is a schematic view. Two coils of aluminum sheet are indicated at 1 and 2, as carried on drums 3 supported by shafts 4. On a shaft 5 are a plurality of drums 6 each carrying a coil of wire or cable 7. It is assumed for the purposes of Fig. 1 that six coils of wire will be carried by six drums mounted to rotate on shaft 5.

The aluminum sheets 1x and 2x and the wire strands 7x move to the right simultaneously, the wire strands being laterally spaced by guiding rolls 8, one set of rolls for each wire, as shown in Fig. 2. The wire strands pass through draw dies indicated at 9 and 10, and thence between the wire brushes 11. From the brushes the drawn and cleansed wire moves on to welding rolls 12.

The aluminum sheets 1x and 2x drawn from the coils thereof may pass through sets of special forming rolls 13 and 14. The forming rolls 13 act upon the top aluminum sheet 1x to corrugate it longitudinally in the manner shown at the top of Fig. 10. The lower set of forming rolls provide deep longitudinal channels in sheet 2x, each for the reception of one of the wires. After leaving the sets of forming rolls 13 and 14, the opposed faces of the sheets are cleaned by wire brushes 15, the sheets being supported by back-up rolls 16. The sheets are led to sets of guiding rolls 17 and then reach a formed scraper 18 which removes any remaining oxide on their inner faces. The lower edge of the scraper will have the channel form of the sheet 2x, and the upper margin of the scraper will have a wavy configuration.

After leaving the scraper zone, the two aluminum sheets, in their form as shown in Fig. 10 will be pressure welded to encase the wire strands, and for this purpose will be passed between the welding rolls 12, the latter having backing rolls 12x, from which the welded composite structure is passed to the slitting wheels 19. Each wire strand will have its aluminum casing with short lips as shown in Fig. 8. To remove the said lips the aluminum encased wire strands are passed through a succession of forming dies 20 which progressively draw the lips 50 down to form a wire-strand-encasing layer of aluminum which, in its tubular form, will have equal thickness throughout. After being cooled the armored wire is wound upon drums or reels 21. Before being wound onto the reels 21 the hot wire may be cooled by sprays of water as indicated by the spray devices 22.

The welding of the aluminum casing elements is accomplished by hot deformation, with the contacting surfaces free from oil and thoroughly cleansed, and preferably slightly roughened by the action of the wire brushes and the scraper blades. An operative temperature range will be 600-900° F. The pressure will exceed several tons and preferably will range from about 25,000 to 70,000 pounds per square inch according to the thickness of the aluminum sheets. The reduction of cross-sectional area should be from 10 to 30 per cent. The aluminum sheets  $1x$ ,  $2x$  may be heated in any suitable manner, but I prefer to heat them by flame pipes or electrical resistance, somewhat close to the welding rolls, and in the drawings I have indicated such flame pipes at 23.

The welding rolls themselves may be heated to a degree high than that acquired by conduction from the hot aluminum sheets, and in order to prevent heat absorption from the sheets and to maintain a predetermined and desired temperature in the sheets themselves at the instant of welding. Also the heated welding rolls may be used to supplement the heat in the aluminum sheets.

The form of the aluminum sheets at the instant of meeting and forming a blanket for the wire strands may be widely varied from the forms shown in Fig. 10. Thus the upper and lower aluminum sheets may be longitudinally corrugated as at the top of Fig. 10, and in reverse. It also will be understood that when the armor is to be relatively thin in thickness pre-forming may be eliminated.

It will be understood that various modifications may be made in the form and arrangement of the elements shown in the drawings as illustrative of the invention, and also in the sequence of steps without departing from the spirit of the invention. Thus, if desired, relatively narrow strips of the sheet can be produced by pre-slitting, and upper and lower tape-like aluminum members will form an encasement for a single wire or cable, my preferred method, however, being as above specified.

Having described my invention, what I claim and desire to secure by Letters Patent, is as follows:

1. The method of continuously applying a non-corrosive metal covering to ferrous cable comprising advancing continuously a plurality of spaced ferrous wire intermediate two continu-

ously advancing relatively thin bands of non-corrosive metal advancing at the same speed as the said wire, heating said thin bands of metal, compressing said heated thin metal bands onto said plurality of wires continuously by means of rollers adapted to receive said wires and heated thin bands of metal, slitting the compressed thin double walled bands intermediate the covered wires to produce a plurality of armored wires having protruding lips on opposite sides of said armored wires, and drawing said armored wire through dies to reduce the said protruding lips to a smooth circular covering.

2. The method of claim 1 wherein the thin band of non-corrosive metal is aluminum and wherein the temperature of the thin metal band is between about 600° F. to about 900° F. and the pressure of compressing the bands onto the ferrous wire is from about 25,000 lbs. to about 70,000 lbs. per square inch.

3. The method of claim 1 wherein the two thin non-corrosive metal bands are complementally shaped to receive a ferrous wire prior to being heated and compressed between rollers.

WILLIAM G. REYNOLDS.

#### REFERENCES CITED

The following references are of record in the file of this patent:

| UNITED STATES PATENTS |               |         |                |
|-----------------------|---------------|---------|----------------|
| Number                | Name          | Country | Date           |
| 155,180               | Coes          |         | Sept. 22, 1874 |
| 867,658               | Hoopes et al. |         | Oct. 8, 1907   |
| 1,124,755             | Lloyd         |         | Jan. 12, 1915  |
| 1,124,763             | Lloyd         |         | Jan. 12, 1915  |
| 1,184,973             | Lloyd         |         | May 30, 1916   |
| 1,326,912             | Cary          |         | Jan. 6, 1920   |
| 1,792,377             | Jordan        |         | Feb. 10, 1931  |
| 1,797,289             | Kotchi        |         | Mar. 24, 1931  |
| 1,812,646             | Burd          |         | June 30, 1931  |
| 1,845,155             | Jordan        |         | Feb. 16, 1932  |
| 1,876,953             | Johnson       |         | Sept. 13, 1932 |
| 2,088,446             | Specht        |         | July 27, 1937  |
| 2,158,656             | Frank         |         | May 16, 1939   |
| 2,375,068             | Bennett       |         | May 1, 1945    |
| 2,382,384             | Cito          |         | Aug. 14, 1945  |

#### FOREIGN PATENTS

| Number  | Country | Date         |
|---------|---------|--------------|
| 513,665 | France  | Nov. 5, 1920 |